

## UNITED STATES PATENT OFFICE

WALTER C. SMITH, OF MOYLAN, PENNSYLVANIA, ASSIGNOR TO ALLIED PROCESS CORPORATION, OF NEW YORK, N. Y., A CORPORATION OF NEW YORK

## PROCESS OF REFINING METALS

No Drawing.

Application filed June 21, 1929. Serial No. 372,797.

This invention relates to a process for the deoxidization and degasification of copper, copper alloys such as brasses and bronzes and other metals and alloys such as zinc and its alloys, nickel, cupro-nickel alloys, iron, steel, and ferrous alloys such as rustless iron, in order to prepare the metal for the production of sound ingots and castings and articles derived therefrom such as bars, rods, wire, etc. The process is especially adapted to the treatment of copper and its alloys and will be more particularly described in connection therewith.

A large number of agents and methods have been proposed for this purpose. Phosphorus and silicon are the agents most commonly employed in the treatment of copper and copper alloys, but while exerting an excellent deoxidizing action are objectionable in that, presumably due to a very small quantity of the agent left in the treated metal, they have a marked deleterious effect upon some of the more important characteristics of the metal, such as electrical conductivity.

Lithium, as I have disclosed in my copending application Serial No. 225,845, filed October 12, 1927, is a superior deoxidizing and degasifying agent for metals, particularly copper and its alloys in that it accomplishes the desired degasification while greatly improving the ductility, malleability, tensile strength and elongation of the metal, and when present in the finished metal in sufficiently small amounts does not appreciably reduce its electrical conductivity. Lithium, however, is relatively expensive and an object of my present invention is to secure all of the advantages incident to the use of lithium as the deoxidizing agent, while at the same time limiting the quantity of lithium required to be used and thereby reducing the cost of the operation. This I accomplish by using a small amount of lithium in conjunction with the use of a less expensive agent such as phosphorus.

Lithium, as I have found, is not only capable of deoxidizing but also apparently is capable of denitrifying, desulfurizing and deposphorizing the metal, and therefore, is capable of completing the deoxidization if it

is not completed by the action of the less expensive agent, and in addition is capable of destroying the deleterious effects produced by the less expensive agent so that a result equal to that produced by the action of lithium alone is accomplished by the use of only a small amount of lithium in conjunction with a less expensive agent. Whether the lithium acts solely to complete the deoxidation or to remove traces of the other deoxidizing agent employed, and the presence of which has a deleterious effect upon the metal, or both has not been determined. A preferred procedure, however, is to use enough of the deoxidizing agent such as phosphorus or silicon to accomplish a complete deoxidization in accordance with well-known practice and then to treat the metal with a very small amount of lithium. As stated, a small amount of lithium left in the metal is not detrimental.

My invention, therefore, contemplates the partial or complete deoxidization and degasification of metals in any well-known way in conjunction with a treatment of the metal with lithium as described in my copending application above referred to. For example copper is treated first in the well-known way with phosphor-copper and then with lithium as such or in the form of an alloy thereof, such as a copper-lithium alloy. The quantity of lithium required will vary widely depending upon the character or purity of the metal treated and the quantity of phosphor-copper used. The quantity should be adjusted so that as little as possible of lithium remains unconsumed and alloyed with the copper. The quantity required cannot readily be determined by analysis but is best determined by tests upon small batches of the metal under treatment, using different amounts until the desired effect is obtained. It may be said that additions of lithium in quantities of the order of .0001% to .05% have been found to be suitable.

As will be understood from the tenor of the foregoing description the lithium is added to the copper at the customary copper refining temperature, that is, from about 1100° C. to about 1250° C.

I claim:

1. In the process of producing sound castings of "copper" the steps which consist in first at least partially degasifying and de-oxidizing the molten metal by the addition thereto of an agent other than lithium and thereafter adding to the molten metal lithium in quantity of from about 0.0001% to about 0.05% at the customary copper-refining tem-  
10 perature of from about 1100° C. to about 1250° C.

2. In the process of producing sound castings of "copper" the steps which consist in first at least partially degasifying and deoxi-  
15 dizing the molten metal by the addition thereto of an agent consisting essentially of phosphorus and thereafter adding to the molten metal lithium in quantity of from about 0.0001% to about 0.05% at the customary  
20 copper-refining temperature of from about 1100° C. to about 1250° C.

In testimony whereof, I affix my signature.  
WALTER C. SMITH.

25

30

35

40

45

50

55

60

65